

Patented Feb. 12, 1924.

1,483,298

# UNITED STATES PATENT OFFICE.

PIERRE GIRIN, OF PARIS, FRANCE, ASSIGNOR TO SOCIETE ANONYME DE COMMENTRY,  
FOURCHAMBAULT & DECAZEVILLE, OF PARIS, FRANCE.

## ALLOY COMPRISING IRON, NICKEL, CHROMIUM, MOLYBDENUM.

No Drawing. Original application filed December 9, 1918, Serial No. 265,985. Divided and this application filed February 8, 1922. Serial No. 535,044.

To all whom it may concern:

Be it known that I, PIERRE GIRIN, a citizen of France, and a resident of Paris, France, have invented new and useful 5 Improvements in Alloys Comprising Iron, Nickel, Chromium, Molybdenum, which is fully set forth in the following specification.

The attainment of an industrial alloy having a high mechanical resistance at high temperatures and capable of definitely preserving its properties, in spite of a prolonged exposure to these temperatures, is a problem which has not yet received a practical solution. In fact, the most resistant steels lose 10 this property rapidly when their temperature is raised from 400 to 500° C. and the hardness conferred by a suitable tempering disappears at the same time as the reheating annuls the action of the treatment.

20 The "high speed" steels certainly preserve their hardness at a temperature higher than the other steels, and after they have been tempered possess a high resistance, even up to a red heat, but besides the drawbacks 25 which result from their fragility and difficulties of a practical nature due to the extremely high temperature of their treatment, they do not present the desired stability when the temperature exceeds 600°; in fact, not 30 only an accidental excess of temperature beyond the regulated value, but even prolonged exposure to this temperature produce a gradual disappearance of the initial hardness and a progressive diminution of resistance. Finally, they are very oxidizable.

In addition, the invention of gas motors, gas turbines and other thermal machines intended to act above the temperature of red heat, and the discovery of chemical synthetic 40 processes using at the same time high temperatures and high pressures, render the realization of a metal possessing certain qualities at high temperature extremely desirable.

The present application, which is a division 45 of my application, Serial No. 265,985, filed December 9, 1918, concerns an alloy of iron, nickel, chromium and molybdenum, and including, perhaps, tungsten or vanadium, cobalt and titanium, easy to obtain in large 50 quantities and capable of being moulded, or otherwise, forged, rolled, wire drawn, worked, without difficulty, possessing at the temperature of 800° a resistance almost equivalent to that of cold iron, non-fragile,

practically inoxidizable at high temperatures, even in a very oxidizing temperature, and at the same time possessing properties which are strictly reversible; by this term I understand that the properties at a given temperature depend solely on that temperature and in no way on the preceding temperatures that have been obtained, nor on an exposure more or less long to the temperature used. The alloy may contain, for example:

|                             | Per cent.  | 65 |
|-----------------------------|------------|----|
| Nickel                      | 60 to 70   |    |
| Chromium                    | 10 to 15   |    |
| Molybdenum                  | 1 to 3     |    |
| Manganese                   | 1 to 2     |    |
| Carbon                      | 0.3 to 0.6 | 70 |
| Iron forming the remainder. |            |    |

Certain variations in the composition may be admitted without introducing important modifications in the quality. The properties 75 are still further improved and the manufacture facilitated by adding to the steel above defined 0.5 to 1 per cent, of vanadium, 0.1 to 0.2 per cent, of titanium, etc.

The alloy thus obtained forms a solid 80 homogeneous solution; no thermal treatment can, consequently, modify its properties. The combined action of chromium and of molybdenum (this last metal being capable of being replaced wholly or partially by tungsten) 85 and, if it is present, of vanadium, is to confer on the alloy of iron and nickel a very high resistance when heated: I can obtain easily 25 to 35 kgs. per sq. mm. with an elastic limit 90 of 20 to 30 kgs. and a coefficient of elongation of 40 per cent at a temperature of 800°, while still preserving a total absence of fragility. These additional elements also render the alloy extremely resistant to the attack of acid 95 vapours, as well as of hot oxidizing and moist gases. This chemical unalterability is of the greatest importance for all applications, since it not only ensures the metal against corrosion, but also ensures the preservation of the initial mechanical properties, in contra-distinction to that which takes place with carbon steels which, when heated for a long time in an atmosphere rich in hydrogen, finally become decarburized and lose their solidity.

This alloy is certainly very suitable for the 10 manufacture of gas turbines or for receptacles, employed in chemical industry, for reactions which take place at high tempera-

ture and at high pressure and which produce corrosive gases or other substances.

Having thus described the nature of the said invention and the best means I know of carrying the same into practical effect, I claim:

A high nickel ferrous alloy containing nickel, 60 to 70 per cent, chromium, 10 to 15 per cent, molybdenum, 1 to 3 per cent, man-

ganese 1 to 2 per cent and carbon, 0.3 to 0.6 per cent, such alloy having at elevated temperatures great mechanical resistance to chemical agents and susceptible of retaining indefinitely its initial properties, notwithstanding prolonged service.

In testimony whereof I have signed this specification.

PIERRE GIRIN.